

# United States Patent [19]

Huang

[11] Patent Number: 4,879,092

[45] Date of Patent: Nov. 7, 1989

[54] **TITANIUM ALUMINUM ALLOYS  
MODIFIED BY CHROMIUM AND NIOBIUM  
AND METHOD OF PREPARATION**

[75] Inventor: Shyh-Chin Huang, Latham, N.Y.

[73] Assignee: General Electric Company,  
Schenectady, N.Y.

[21] Appl. No.: 201,984

[22] Filed: Jun. 3, 1988

[51] Int. Cl.<sup>4</sup> ..... C22C 14/00; C21D 1/00  
[52] U.S. Cl. ..... 420/418; 75/245;

148/12.7 B; 148/133; 428/614

[58] Field of Search ..... 420/418; 148/133, 12.7 B;  
75/245; 428/614

[56] **References Cited**

**U.S. PATENT DOCUMENTS**

3,203,794 8/1965 Jaffee et al. ..... 420/418  
4,294,615 10/1981 Blackburn et al. ..... 148/133  
4,639,281 1/1987 Sastry et al. ..... 420/418  
4,661,316 4/1980 Hashimoto et al. ..... 420/418  
4,746,374 5/1988 Froes et al. ..... 428/614

**FOREIGN PATENT DOCUMENTS**

0220571 7/1957 Australia ..... 420/418

**OTHER PUBLICATIONS**

Baker et al., Journal of Metals, Feb. 1988, pp. 28-31.  
Whang et al., in ASM Symposium, Oct. 1986, Orlando,  
Fla., pp. 1-7.  
Lipsitt, H. A., "Titanium Aluminides—An Overview",

Mat. Res. Soc. Symposium Proc., vol. 39, Materials  
Research Society, (1985), pp. 351-364.

Sastry et al., Met. Trans. 8A, "Fatigue Deformation of  
TiAl Base Alloys", (1977), pp. 299-308.

Izvestiya Akademii Nauk SSSR, Metally, No. 3, (1984),  
pp. 164-168—Transl., ("Deformation & Failure in  
Titanium Aluminide", (1985), pp. 157-161).

Martin, P. L./Lipsitt, H. A./Nuhfer, N. T./Williams, J.  
C., "The Effects of Alloying on the Microstructure and  
Properties of Ti<sub>3</sub>Al and TiAl", Titanium 80, (published  
by The American Society of Metals, Warrendale, Pa.),  
vol. 2, (1980), pp. 1245-1254.

Tsujimoto, T., "Research, Development, and Prospects  
of TiAl Intermetallic Compound Alloys", Titanium &  
Zirconium, vol. 33, No. 3, 159, (Jul. 1985), pp. 1-19.

*Primary Examiner*—Upendra Roy  
*Attorney, Agent, or Firm*—Paul E. Rochford; James C.  
Davis, Jr.; James Magee, Jr.

[57] **ABSTRACT**

A TiAl composition is prepared to have high strength  
and to have improved ductility by altering the atomic  
ratio of the titanium and aluminum to have what has  
been found to be a highly desirable effective aluminum  
concentration by addition of chromium and niobium  
according to the approximate formula —Ti<sub>50.46</sub>Al<sub>46.50</sub>Cr<sub>2</sub>Nb<sub>2</sub>.

18 Claims, 5 Drawing Sheets





FIG. 1



FIG. 2



FIG. 3



FIG. 4

## Ti - 48Al - 2Cr - 2Nb R. T. TENSILE TEST



FIG. 5

## Ti - 48Al - 2Cr - 2Nb R. T. TENSILE TEST



FIG. 6

**TITANIUM ALUMINUM ALLOYS MODIFIED BY CHROMIUM AND NIOBIUM AND METHOD OF PREPARATION**

**CROSS REFERENCE TO RELATED APPLICATIONS**

The subject application relates to copending applications as follows:

Ser. Nos. 138,476; 138,481; 138,486; 138,407; 138,408; 07/293,035 (RD-18,643), filed 1-3-1989; 07/219,106 (RD-18,688), filed 7/14/85 and 07/252,622 (RD-18,829), filed 10/3/88.

The texts of these related applications are incorporated herein by reference.

**BACKGROUND OF THE INVENTION**

The present invention relates generally to alloys of titanium and aluminum. More particularly it relates to gamma alloys of titanium and aluminum which have been modified both with respect to stoichiometric ratio and with respect to chromium and niobium addition.

It is known that as aluminum is added to titanium metal in greater and greater proportions the crystal form of the resultant titanium aluminum composition changes. Small percentages of aluminum go into solid solution in titanium and the crystal form remains that of alpha titanium. At higher concentrations of aluminum (including about 25 to 35 atomic %) an intermetallic compound  $Ti_3Al$  is formed. The  $Ti_3Al$  has an ordered hexagonal crystal form called alpha-2. At still higher concentrations of aluminum (including the range of 50 to 60 atomic % aluminum) another intermetallic compound,  $TiAl$ , is formed having an ordered tetragonal crystal form called gamma.

The alloy of titanium and aluminum having a gamma crystal form, and a stoichiometric ratio of approximately one, is an intermetallic compound having a high modulus, a low density, a high thermal conductivity, favorable oxidation resistance, and good creep resistance. The relationship between the modulus and temperature for  $TiAl$  compounds to other alloys of titanium and in relation to nickel base superalloys is shown in FIG. 1. As is evident from the figure the  $TiAl$  has the best modulus of any of the titanium alloys. Not only is the  $TiAl$  modulus higher at higher temperature but the rate of decrease of the modulus with temperature increase is lower for  $TiAl$  than for the other titanium alloys. Moreover, the  $TiAl$  retains a useful modulus at temperatures above those at which the other titanium alloys become useless. Alloys which are based on the  $TiAl$  intermetallic compound are attractive lightweight materials for use where high modulus is required at high temperatures and where good environmental protection is also required.

One of the characteristics of  $TiAl$  which limits its actual application to such uses is a brittleness which is found to occur at room temperature. Also the strength of the intermetallic compound at room temperature needs improvement before the  $TiAl$  intermetallic compound can be exploited in structural component applications. Improvements of the  $TiAl$  intermetallic compound to enhance ductility and/or strength at room temperature are very highly desirable in order to permit use of the compositions at the higher temperatures for which they are suitable.

With potential benefits of use at light weight and at high temperatures, what is most desired in the  $TiAl$

compositions which are to be used is a combination of strength and ductility at room temperature. A minimum ductility of the order of one percent is acceptable for some applications of the metal composition but higher ductilities are much more desirable. A minimum strength for a composition to be useful is about 50 ksi or about 350 MPa. However, materials having this level of strength are of marginal utility and higher strengths are often preferred for some applications.

The stoichiometric ratio of  $TiAl$  compounds can vary over a range without altering the crystal structure. The aluminum content can vary from about 50 to about 60 atom percent. The properties of  $TiAl$  compositions are subject to very significant changes as a result of relatively small changes of one percent or more in the stoichiometric ratio of the titanium and aluminum ingredients. Also the properties are similarly affected by the addition of relatively similar small amounts of ternary elements.

I have now discovered that further improvements can be made in the gamma  $TiAl$  intermetallic compounds by incorporating therein a combination of additive elements so that the composition not only contains a ternary additive element but also a quaternary additive element.

Furthermore I have discovered that the composition including the quaternary additive element has a uniquely desirable combination of properties which include a desirably high ductility and a valuable oxidation resistance.

**PRIOR ART**

There is extensive literature on the compositions of titanium aluminum including the  $Ti_3Al$  intermetallic compound, the  $TiAl$  intermetallic compounds and the  $TiAl_3$  intermetallic compound. A U.S. Pat. No. 4,294,615, entitled "Titanium Alloys of the  $TiAl$  Type" contains an extensive discussion of the titanium aluminide type alloys including the  $TiAl$  intermetallic compound. As is pointed out in the patent in column 1 starting at line 50 in discussing  $TiAl$ 's advantages and disadvantages relative to  $Ti_3Al$ :

"It should be evident that the  $TiAl$  gamma alloy system has the potential for being lighter inasmuch as it contains more aluminum. Laboratory work in the 1950's indicated that titanium aluminide alloys had the potential for high temperature use to about 1000° C. But subsequent engineering experience with such alloys was that, while they had the requisite high temperature strength, they had little or no ductility at room and moderate temperatures, i.e., from 20° to 550° C. Materials which are too brittle cannot be readily fabricated, nor can they withstand infrequent but inevitable minor service damage without cracking and subsequent failure. They are not useful engineering materials to replace other base alloys."

It is known that the alloy system  $TiAl$  is substantially different from  $Ti_3Al$  (as well as from solid solution alloys of Ti) although both  $TiAl$  and  $Ti_3Al$  are basically ordered titanium aluminum intermetallic compounds. As the '615 patent points out at the bottom of column 1:

"Those well skilled recognize that there is a substantial difference between the two ordered phases.

Alloying and transformational behavior of  $Ti_3Al$  resemble those of titanium as the hexagonal crystal structures are very similar. However, the compound  $TiAl$  has a tetragonal arrangement of atoms and thus rather different alloying characteristics. Such a distinction is often not recognized in the earlier literature."

The '615 patent does describe the alloying of  $TiAl$  with vanadium and carbon to achieve some property improvements in the resulting alloy.

The '615 patent also discloses in Table 2 alloy  $T_2A-112$  which is a composition in atomic percent of  $Ti-45Al-5.0Nb$  but the patent does not describe the composition as having any beneficial properties.

A number of technical publications dealing with the titanium aluminum compounds as well as with the characteristics of these compounds are as follows:

1. E. S. Bumps, H. D. Kessler, and M. Hansen, "Titanium-Aluminum System", *Journal of Metals*, June, 1952, pp. 609-614, TRANSACTIONS AIME, Vol. 194.

2. H. R. Ogden, D. J. Maykuth, W. L. Finlay, and R. I. Jaffee, "Mechanical Properties of High Purity  $Ti-Al$  Alloys", *Journal of Metals*, February, 1953, pp. 267-272, TRANSACTIONS AIME, Vol. 197.

3. Joseph B. McAndrew, and H. D. Kessler, "Ti-36 Pct Al as a Base for High Temperature Alloys", *Journal of Metals*, October, 1956, pp. 1348-1353, TRANSACTIONS AIME, Vol. 206.

The McAndrew reference discloses work under way toward development of a  $TiAl$  intermetallic gamma alloy. In Table II, McAndrew reports alloys having ultimate tensile strength of between 33 and 49 ksi as adequate "where designed stresses would be well below this level". This statement appears immediately above Table II. In the paragraph above Table IV, McAndrew states that tantalum, silver and (niobium) columbium have been found useful alloys in inducing the formation of thin protective oxides on alloys exposed to temperatures of up to  $1200^{\circ}C$ . FIG. 4 of McAndrew is a plot of the depth of oxidation against the nominal weight percent of niobium exposed to still air at  $1200^{\circ}C$ . for 96 hours. Just above the summary on page 1353 a sample of titanium alloy containing 7 weight % columbium (niobium) is reported to have displayed a 50% higher rupture stress properties than the Ti-36%Al used for comparison.

#### BRIEF DESCRIPTION OF THE INVENTION

One object of the present invention is to provide a method of forming a titanium aluminum intermetallic compound having improved ductility and related properties at room temperature.

Another object is to improve the properties of titanium aluminum intermetallic compounds at low and intermediate temperatures.

Another object is to provide an alloy of titanium and aluminum having improved properties and processability at low and intermediate temperatures.

Another object is to improve the combination of ductility and oxidation resistance of  $TiAl$  base compositions.

Still another object is to improve the oxidation resistance of  $TiAl$  compositions.

Yet another object is to make improvements in a set of strength, ductility and oxidation resistance properties.

Other objects will be in part apparent and in part pointed out in the description which follows.

In one of its broader aspects the objects of the present invention are achieved by providing a nonstoichiometric  $TiAl$  base alloy, and adding a relatively low concentration of chromium and a low concentration of niobium to the nonstoichiometric composition. The addition may be followed by rapidly solidifying the chromium-containing nonstoichiometric  $TiAl$  intermetallic compound. Addition of chromium in the order of approximately 1 to 3 atomic percent and of niobium to the extent of 1 to 5 atomic percent is contemplated.

The rapidly solidified composition may be consolidated as by isostatic pressing and extrusion to form a solid composition of the present invention.

The alloy of this invention may also be produced in ingot form and may be processed by ingot metallurgy.

#### BRIEF DESCRIPTION OF THE DRAWINGS

FIG. 1 is a graph illustrating the relationship between modulus and temperature for an assortment of alloys.

FIG. 2 is a graph illustrating the relationship between load in pounds and crosshead displacement in mils for  $TiAl$  compositions of different stoichiometry tested in 4-point bending.

FIG. 3 is a graph similar to that of FIG. 2 but illustrating the relationship of FIG. 2 for  $Ti_{50}Al_{48}Cr_2$ .

FIG. 4 is a graph displaying comparative oxidation resistance properties.

FIG. 5 is a bar graph displaying strength in ksi for samples given of different heat treatments.

FIG. 6 is a similar graph displaying ductility in relation to temperature of heat treatment.

#### DETAILED DESCRIPTION OF THE INVENTION

##### EXAMPLES 1-3

Three individual melts were prepared to contain titanium and aluminum in various stoichiometric ratios approximating that of  $TiAl$ . The compositions, annealing temperatures and test results of tests made on the compositions are set forth in Table I.

For each example the alloy was first made into an ingot by electro arc melting. The ingot was processed into ribbon by melt spinning in a partial pressure of argon. In both stages of the melting, a water-cooled copper hearth was used as the container for the melt in order to avoid undesirable melt-container reactions.

Also care was used to avoid exposure of the hot metal to oxygen because of the strong affinity of titanium for oxygen.

The rapidly solidified ribbon was packed into a steel can which was evacuated and then sealed. The can was then hot isostatically pressed (HIPped) at  $950^{\circ}C$ . ( $1740^{\circ}F$ .) for 3 hours under a pressure of 30 ksi. The HIPping can was machined off the consolidated ribbon plug. The HIPped sample was a plug about one inch in diameter and three inches long.

The plug was placed axially into a center opening of a billet and sealed therein. The billet was heated to  $975^{\circ}C$ . ( $1787^{\circ}F$ .) and is extruded through a die to give a reduction ratio of about 7 to 1. The extruded plug was removed from the billet and was heat treated.

The extruded samples were then annealed at temperatures as indicated in Table I for two hours. The annealing was followed by aging at  $1000^{\circ}C$ . for two hours. Specimens were machined to the dimension of

$1.5 \times 3 \times 25.4$  mm ( $0.060 \times 0.120 \times 1.0$  in) for four point bending tests at room temperature. The bending tests

$1300^\circ$  C. and further data on these samples in particular is given in FIG. 2.

TABLE I

| Ex. No. | Gamma Alloy No. | Composit. (at %)                  | Anneal Temp. ( $^\circ$ C.) | Yield Strength (ksi) | Fracture Strength (ksi) | Outer Fiber Strain (%) |
|---------|-----------------|-----------------------------------|-----------------------------|----------------------|-------------------------|------------------------|
| 1       | 83              | Ti <sub>54</sub> Al <sub>46</sub> | 1250                        | 131                  | 132                     | 0.1                    |
|         |                 |                                   | 1300                        | 111                  | 120                     | 0.1                    |
|         |                 |                                   | 1350                        | —*                   | 58                      | 0                      |
| 2       | 12              | Ti <sub>52</sub> Al <sub>48</sub> | 1250                        | 130                  | 180                     | 1.1                    |
|         |                 |                                   | 1300                        | 98                   | 128                     | 0.9                    |
|         |                 |                                   | 1350                        | 88                   | 122                     | 0.9                    |
| 3       | 85              | Ti <sub>50</sub> Al <sub>50</sub> | 1250                        | 83                   | 92                      | 0.3                    |
|         |                 |                                   | 1300                        | 93                   | 97                      | 0.3                    |
|         |                 |                                   | 1350                        | 78                   | 88                      | 0.4                    |

\*No measurable value was found because the sample lacked sufficient ductility to obtain a measurement.

were carried out in a 4-point bending fixture having an inner span of 10 mm (0.4 in) and an outer span of 20 mm (0.8 in). The load-crosshead displacement curves were recorded. Based on the curves developed the following properties are defined:

1. Yield strength is the flow stress at a cross head displacement of one thousandth of an inch. This amount of cross head displacement is taken as the first evidence of plastic deformation and the transition from elastic deformation to plastic deformation. The measurement of yield and/or fracture strength by conventional compression or tension methods tends to give results which are lower than the results obtained by four point bending as carried out in making the measurements reported herein. The higher levels of the results from four point bending measurements should be kept in mind when comparing these values to values obtained by the conventional compression or tension methods. However, the comparison of measurements results in the examples herein is between four point bending tests for all samples measured and such comparisons are quite valid in establishing the differences in strength properties resulting from differences in composition or in processing of the compositions.

2. Fracture strength is the stress to fracture.

3. Outer fiber strain is the quantity of  $9.71 \text{ hd}$ , where  $h$  is the specimen thickness in inches and  $d$  is the cross head displacement of fracture in inches. Metallurgically, the value calculated represents the amount of plastic deformation experienced at the outer surface of the bending specimen at the time of fracture.

The results are listed in the following Table I. Table I contains data on the properties of samples annealed at

20 It is evident from the data of this table that alloy 12 for Example 2 exhibited the best combination of properties. This confirms that the properties of Ti-Al compositions are very sensitive to the Ti/Al atomic ratios and to the heat treatment applied. Alloy 12 was selected as the base alloy for further property improvements based on further experiments which were performed as described below.

25 It is also evident that the anneal at temperatures between  $1250^\circ$  C. and  $1350^\circ$  C. results in the test specimens having desirable levels of yield strength, fracture strength and outer fiber strain. However, the anneal at  $1400^\circ$  C. results in a test specimen having a significantly lower yield strength (about 20% lower); lower fracture strength (about 30% lower) and lower ductility (about 78% lower) than a test specimen annealed at  $1350^\circ$  C. The sharp decline in properties is due to a dramatic change in microstructure due in turn to an extensive beta transformation at temperatures appreciably above  $1350^\circ$  C.

#### EXAMPLES 4-13

30 Ten additional individual melts were prepared to contain titanium and aluminum in designated atomic ratios as well as additives in relatively small atomic percents.

35 Each of the samples was prepared as described above with reference to Examples 1-3.

40 The compositions, annealing temperatures, and test results of tests made on the compositions are set forth in Table II in comparison to alloy 12 as the base alloy for this comparison.

TABLE II

| Ex. No. | Gamma Alloy No. | Composit. (at %)                                  | Anneal Temp. ( $^\circ$ C.) | Yield Strength (ksi) | Fracture Strength (ksi) | Outer Fiber Strain (%) |
|---------|-----------------|---------------------------------------------------|-----------------------------|----------------------|-------------------------|------------------------|
| 2       | 12              | Ti <sub>52</sub> Al <sub>48</sub>                 | 1250                        | 130                  | 180                     | 1.1                    |
|         |                 |                                                   | 1300                        | 98                   | 128                     | 0.9                    |
| 4       | 22              | Ti <sub>50</sub> Al <sub>47</sub> Ni <sub>3</sub> | 1200                        | —*                   | 131                     | 0                      |
|         |                 |                                                   | 1300                        | 92                   | 117                     | 0.5                    |
| 5       | 24              | Ti <sub>52</sub> Al <sub>46</sub> Ag <sub>2</sub> | 1200                        | —*                   | 114                     | 0                      |
|         |                 |                                                   | 1300                        | —*                   | 117                     | 0.5                    |
| 6       | 25              | Ti <sub>50</sub> Al <sub>48</sub> Cu <sub>2</sub> | 1250                        | —*                   | 83                      | 0                      |
|         |                 |                                                   | 1300                        | 80                   | 107                     | 0.8                    |
| 7       | 32              | Ti <sub>54</sub> Al <sub>45</sub> Hf <sub>1</sub> | 1250                        | 130                  | 136                     | 0.1                    |
|         |                 |                                                   | 1300                        | 72                   | 77                      | 0.1                    |
| 8       | 41              | Ti <sub>52</sub> Al <sub>44</sub> Pt <sub>4</sub> | 1250                        | 132                  | 150                     | 0.3                    |
|         |                 |                                                   | 1300                        | 136                  | 149                     | 0.1                    |
| 9       | 45              | Ti <sub>51</sub> Al <sub>47</sub> C <sub>2</sub>  | 1250                        | —*                   | 89                      | 0                      |
|         |                 |                                                   | 1300                        | —*                   | 81                      | 0                      |
| 10      | 57              | Ti <sub>50</sub> Al <sub>48</sub> Fe <sub>2</sub> | 1250                        | —*                   | 89                      | 0                      |
|         |                 |                                                   | 1300                        | —*                   | 81                      | 0                      |

TABLE II-continued

| Ex. No. | Gamma Alloy No. | Composit. (at %)                                      | Anneal Temp. (°C.) | Yield Strength (ksi) | Fracture Strength (ksi) | Outer Fiber Strain (%) |
|---------|-----------------|-------------------------------------------------------|--------------------|----------------------|-------------------------|------------------------|
| 11      | 82              | Ti <sub>50</sub> Al <sub>48</sub> Mo <sub>2</sub>     | 1350               | 86                   | 111                     | 0.5                    |
|         |                 |                                                       | 1250               | 128                  | 140                     | 0.2                    |
|         |                 |                                                       | 1300               | 110                  | 136                     | 0.5                    |
|         |                 |                                                       | 1350               | 80                   | 95                      | 0.1                    |
| 12      | 39              | Ti <sub>50</sub> Al <sub>46</sub> Mo <sub>4</sub>     | 1200               | —*                   | 143                     | 0                      |
|         |                 |                                                       | 1250               | 135                  | 154                     | 0.3                    |
|         |                 |                                                       | 1300               | 131                  | 149                     | 0.2                    |
| 13      | 20              | Ti <sub>49.5</sub> Al <sub>49.5</sub> Er <sub>1</sub> | +                  | +                    | +                       | +                      |

\*See asterisk note to Table I.

+ Material fractured during machining to prepare test specimens.

For Examples 4 and 5 heat treated at 1200° C., the yield strength was unmeasurable as the ductility was found to be essentially nil. For the specimen of Example 5 which was annealed at 1300° C., the ductility increased, but it was still undesirably low.

For Example 6 the same was true for the test specimens annealed at 1250° C. For the specimens of Example 6 which were annealed at 1300° and 1350° C. the ductility was significant but the yield strength was low.

None of the test specimens of the other Examples 25 were found to have any significant level of ductility.

It is evident from the results listed in Table II that the sets of parameters involved in preparing compositions for testing are quite complex and interrelated. One parameter is the atomic ratio of the titanium relative to that of aluminum. From the data plotted in FIG. 2 it is evident that the stoichiometric ratio or non-stoichiometric ratio has a strong influence on the test properties which formed for different compositions.

Another set of parameters is the additive chosen to be included into the basic TiAl composition. A first parameter of this set concerns whether a particular additive acts as a substituent for titanium or for aluminum. A specific metal may act in either fashion and there is no simple rule by which it can be determined which role an additive will play. The significance of this parameter is evident if we consider addition of some atomic percentage of additive X.

If X acts as a titanium substituent then a composition Ti<sub>48</sub>Al<sub>48</sub>X<sub>4</sub> will give an effective aluminum concentration of 48 atomic percent and an effective titanium concentration of 52 atomic percent.

If by contrast the X additive acts as an aluminum substituent then the resultant composition will have an effective aluminum concentration of 52 percent and an effective titanium concentration of 48 atomic percent.

Accordingly the nature of the substitution which takes place is very important but is also highly unpredictable.

Another parameter of this set is the concentration of the additive.

Still another parameter evident from Table II is the annealing temperature. The annealing temperature which produces the best strength properties for one additive can be seen to be different for a different additive. This can be seen by comparing the results set forth in Example 6 with those set forth in Example 7.

In addition there may be a combined concentration and annealing effect for the additive so that optimum property enhancement, if any enhancement is found, can occur at a certain combination of additive concentration and annealing temperature so that higher and lower concentrations and/or annealing temperatures

are less effective in providing a desired property improvement.

The content of Table II makes clear that the results obtainable from addition of a ternary element to a non-stoichiometric TiAl composition are highly unpredictable and that most test results are unsuccessful with respect to ductility or strength or to both.

#### EXAMPLES 14-17

A further parameter of the titanium aluminide alloys which include additives is that combinations of additives do not necessarily result in additive combinations of the individual advantages resulting from the individual and separate inclusion of the same additives.

Four additional TiAl based samples were prepared as described above with reference to Examples 1-3 to contain individual additions of vanadium, niobium and tantalum as listed in Table III. These compositions are the optimum compositions reported in copending applications Ser. Nos. 138,476; 138,408; and 138,485, respectively.

The fourth composition is a composition which combines the vanadium, niobium and tantalum into a single alloy designated in Table III to be alloy 48.

From Table III it is evident that the individual additions vanadium, niobium and tantalum are able on an individual basis in Examples 14, 15 and 16 to each lend substantial improvement to the base TiAl alloy. However, these same additives when combined into a single combination alloy do not result in a combination of the individual improvements in an additive fashion. Quite the reverse is the case.

In the first place the alloy 48 which was annealed at the 1350° C. temperature used in annealing the individual alloys was found to result in production of such a brittle material that it fractured during machining to prepare test specimens.

Secondly the results which are obtained for the combined additive alloy annealed at 1250° C. are very inferior to those which are obtained for the separate alloys containing the individual additives.

In particular with reference to the ductility it is evident that the vanadium was very successful in substantially improving the ductility in the alloy 14 of Example 60 14. However, when the vanadium is combined with the other additives in alloy 48 of Example 17 the ductility improvement which might have been achieved is not achieved at all. In fact the ductility of the base alloy is reduced to a value of 0.1.

Further with reference to the oxidation resistance the niobium additive of alloy 40 clearly shows a very substantial improvement in the 4 mg/cm<sup>2</sup> weight loss of alloy 40 as compared to the 31 mg/cm<sup>2</sup> weight loss of

the base alloy. The test of oxidation, and the complementary test of oxidation resistance, involves heating a sample to be tested at a temperature of 982° C. for a period of 48 hours. After the sample has cooled it is scraped to remove any oxide scale. By weighing the sample both before and after the heating and scraping a weight difference can be determined. Weight loss is determined in mg/cm<sup>2</sup> by dividing the total weight loss in grams by the surface area of the specimen in square centimeters. This oxidation test is the one used for all measurements of oxidation or oxidation resistance as set forth in this application.

For the alloy 60 with the tantalum additive the weight loss for a sample annealed at 1325° C. was determined to be 2 mg/cm<sup>2</sup> and this is again compared to the 31 mg/cm<sup>2</sup> weight loss for the base alloy. In other words on an individual additive basis both niobium and tantalum additives were very effective in improving oxidation resistance of the base alloy.

However as is evident from Example 17 results listed in Table III alloy 48 which contained all three additives, vanadium, niobium and tantalum in combination, the oxidation is increased to about double that of the base alloy. This is seven times greater than alloy 40 which contained the niobium additive above and about 15 times greater than alloy 60 which contained the tantalum additive alone.

TABLE III

| Example Number | Alloy Number | Composition (at %)                                                               | Annealing Temperature (°C.) | Yield Strength (ksi) | Fracture Strength (ksi) | Outer Fiber Strain (%) | Weight Loss After 48 hrs. at 982° C. (mg/cm <sup>2</sup> ) |
|----------------|--------------|----------------------------------------------------------------------------------|-----------------------------|----------------------|-------------------------|------------------------|------------------------------------------------------------|
| 2              | 12           | Ti <sub>52</sub> Al <sub>48</sub>                                                | 1250                        | 130                  | 180                     | 1.1                    | —*                                                         |
|                |              |                                                                                  | 1300                        | 98                   | 128                     | 0.9                    | —*                                                         |
|                |              |                                                                                  | 1350                        | 88                   | 122                     | 0.8                    | 31                                                         |
| 14             | 14           | Ti <sub>49</sub> Al <sub>48</sub> V <sub>3</sub>                                 | 1300                        | 94                   | 145                     | 1.6                    | 27                                                         |
|                |              |                                                                                  | 1350                        | 84                   | 136                     | 1.5                    | —*                                                         |
| 15             | 40           | Ti <sub>50</sub> Al <sub>46</sub> Nb <sub>4</sub>                                | 1250                        | 136                  | 167                     | 0.5                    | —*                                                         |
|                |              |                                                                                  | 1300                        | 124                  | 176                     | 1.0                    | 4                                                          |
|                |              |                                                                                  | 1350                        | 86                   | 100                     | 0.1                    | —*                                                         |
| 16             | 60           | Ti <sub>48</sub> Al <sub>48</sub> Ta <sub>4</sub>                                | 1250                        | 120                  | 147                     | 1.1                    | —*                                                         |
|                |              |                                                                                  | 1300                        | 106                  | 141                     | 1.3                    | —*                                                         |
|                |              |                                                                                  | 1325                        | —*                   | —*                      | —*                     | 2                                                          |
|                |              |                                                                                  | 1350                        | 97                   | 137                     | 1.5                    | —*                                                         |
|                |              |                                                                                  | 1400                        | 72                   | 92                      | 0.2                    | —*                                                         |
| 17             | 48           | Ti <sub>49</sub> Al <sub>45</sub> V <sub>2</sub> Nb <sub>2</sub> Ta <sub>2</sub> | 1250                        | 106                  | 107                     | 0.1                    | 60                                                         |
|                |              |                                                                                  | 1350                        | +                    | +                       | +                      | —*                                                         |

\*Not measured.

+Material fractured during machining to prepare test specimen.

The individual advantages or disadvantages which result from the use of individual additives repeat reliably as these additions are used individually over and over again. However, when additives are used in combination the effect of an additive in the combination in a base alloy can be quite different from the effect of the additive when used individually and separately in the same base alloy. Thus, it has been discovered that addition of vanadium is beneficial to the ductility of titanium aluminum compositions and this is disclosed and discussed in the copending application for patent Ser. No. 138,476. Further, one of the additives which has been found to be beneficial to the strength of the TiAl base and which is described in copending application Ser. No. 138,408, filed Dec. 28, 1987 as discussed above is the additive niobium. In addition it has been shown by the McAndrew paper discussed above that the individual addition of niobium additive to TiAl base alloy can improve oxidation resistance. Similarly the individual addition of tantalum is taught by McAndrew as assisting

than some combined beneficial overall gain of properties.

However from Table 3 above it is evident that the alloy containing the combination of the vanadium, niobium and tantalum additions has far worse oxidation resistance than the base TiAl 12 alloy of Example 2. Here again the combined inclusion of additives which improve a property on a separate and individual basis have been found to result in a net loss in the very property which is improved when the additives are included on a separate and individual basis.

#### EXAMPLES 18 through 23

Six additional samples were prepared as described above with reference to Examples 1-3 to contain chromium modified titanium aluminide having compositions respectively as listed in Table IV.

Table IV summarizes the bend test results on all of the alloys both standard and modified under the various heat treatment conditions deemed relevant.

in improving oxidation resistance. Furthermore, in copending application Ser. No. 138,485 it is disclosed that addition of tantalum results in improvements in ductility.

In other words, it has been found that vanadium can individually contribute advantageous ductility improvements to titanium aluminum compound and that tantalum can individually contribute to ductility and oxidation improvements. It has been found separately that niobium additives can contribute beneficially to the strength and oxidation resistance properties of titanium aluminum. However, the applicant has found as is indicated from this Example 17, that when vanadium, tantalum, and niobium are used together and are combined as additives in an alloy composition, the alloy composition is not benefitted by the additions but rather there is a net decrease or loss in properties of the TiAl which contains the niobium, the tantalum, and the vanadium additives. This is evident from Table III.

From this it is evident that while it may seem that if two or more additive elements individually improve TiAl that their use together should render further improvements to the TiAl, it is found nevertheless that such additions are highly unpredictable and that, in fact, for the combined additions of vanadium, niobium and tantalum a net loss of properties result from the combined use of the combined additives together rather

TABLE IV

## FOUR-POINT BEND PROPERTIES OF Cr-MODIFIED TiAl ALLOYS

| Ex. | Gammas<br>Alloy<br>Number | Compo-<br>sition<br>(at %)                        | Annealing<br>Temperature<br>(°C.) | Yield<br>Strength<br>(ksi) | Fracture<br>Strength<br>(ksi) | Outer<br>Fiber<br>Strain<br>(%) |
|-----|---------------------------|---------------------------------------------------|-----------------------------------|----------------------------|-------------------------------|---------------------------------|
| 2   | 12                        | Ti <sub>52</sub> Al <sub>48</sub>                 | 1250                              | 130                        | 180                           | 1.0                             |
|     |                           |                                                   | 1300                              | 98                         | 128                           | 0.9                             |
|     |                           |                                                   | 1350                              | 88                         | 122                           | 0.9                             |
| 18  | 38                        | Ti <sub>52</sub> Al <sub>46</sub> Cr <sub>2</sub> | 1250                              | 113                        | 170                           | 1.6                             |
|     |                           |                                                   | 1300                              | 91                         | 123                           | 0.4                             |
|     |                           |                                                   | 1350                              | 71                         | 89                            | 0.2                             |
| 19  | 80                        | Ti <sub>50</sub> Al <sub>48</sub> Cr <sub>2</sub> | 1250                              | 97                         | 131                           | 1.2                             |
|     |                           |                                                   | 1300                              | 89                         | 135                           | 1.5                             |
|     |                           |                                                   | 1350                              | 93                         | 108                           | 0.2                             |
| 20  | 87                        | Ti <sub>48</sub> Al <sub>50</sub> Cr <sub>2</sub> | 1250                              | 108                        | 122                           | 0.4                             |
|     |                           |                                                   | 1300                              | 106                        | 121                           | 0.3                             |
|     |                           |                                                   | 1350                              | 100                        | 125                           | 0.7                             |
| 21  | 49                        | Ti <sub>50</sub> Al <sub>46</sub> Cr <sub>4</sub> | 1250                              | 104                        | 107                           | 0.1                             |
|     |                           |                                                   | 1300                              | 90                         | 116                           | 0.3                             |
| 22  | 79                        | Ti <sub>48</sub> Al <sub>48</sub> Cr <sub>4</sub> | 1250                              | 122                        | 142                           | 0.3                             |
|     |                           |                                                   | 1300                              | 111                        | 135                           | 0.4                             |
|     |                           |                                                   | 1350                              | 61                         | 74                            | 0.2                             |
| 23  | 88                        | Ti <sub>46</sub> Al <sub>50</sub> Cr <sub>4</sub> | 1250                              | 128                        | 139                           | 0.2                             |
|     |                           |                                                   | 1300                              | 122                        | 133                           | 0.2                             |
|     |                           |                                                   | 1350                              | 113                        | 131                           | 0.3                             |

The results listed in Table IV offer further evidence of the criticality of a combination of factors in determining the effects of alloying additions or doping additions on the properties imparted to a base alloy. For example the alloy 80 shows a good set of properties for a 2 atomic percent addition of chromium. One might expect further improvement from further chromium addition. However the addition of 4 atomic percent chromium to alloys having three different TiAl atomic ratios demonstrates that the increase in concentration of an additive found to be beneficial at lower concentrations does not follow the simple reasoning that if some is good more must be better. And in fact for the chromium additive just the opposite is true and demonstrates that where some is good, more is bad.

As is evident from Table IV each of the alloys 49, 79 and 88 which contain "more" (4 atomic percent) chromium shows inferior strength and also inferior outer fiber strain (ductility) compared with the base alloy.

By contrast, alloy 38 of Example 18 contains 2 atomic percent of additive and shows only slightly reduced strength but greatly improved ductility. Also it can be observed that the measured outer fiber strain of alloy 38 varied significantly with the heat treatment conditions. A remarkable increase in the outer fiber strain was achieved by annealing at 1250° C. Reduced strain was observed when annealing at higher temperatures. Similar improvements were observed for alloy 80 which also contained only 2 atomic percent of additive although the annealing temperature was 1300° C. for the highest ductility achieved.

For Example 20 alloy 87 employed the level of 2 atomic percent of chromium but the concentration of aluminum is increased to 50 atomic percent. The higher aluminum concentration leads to a small reduction in the ductility from the ductility measured for the two percent chromium compositions with aluminum in the 46 to 48 atomic percent range. For alloy 87 the optimum heat treatment temperature was found to be about 1350° C.

From Examples 18, 19 and 20 which each contained 2 atomic percent additive it was observed that the optimum annealing temperature increased with increasing aluminum concentration.

From this data it was determined that alloy 38 which has been heat treated at 1250° C., had the best combination of room temperature properties. Note that the optimum annealing temperature for alloy 38 with 46 at. % aluminum was 1250° C. but the optimum for alloy 80 with 48 at. % aluminum was 1300° C.

These remarkable increases in the ductility of alloy 38 on treatment at 1250° C. and of alloy 80 on heat treatment at 1300° C. were unexpected as is explained in the copending application for Ser. No. 138,485 filed Dec. 28, 1987.

What is clear from the data contained in Table IV is that the modification of TiAl compositions to improve the properties of the compositions is a very complex and unpredictable undertaking. For example, it is evident that chromium at 2 atomic percent level does very substantially increase the ductility of the composition where the atomic ratio of TiAl is in an appropriate range and where the temperature of annealing of the composition is in an appropriate range for the chromium additions. It is also clear from the data of Table IV that although one might expect greater effect in improving properties by increasing the level of additive that just the reverse is the case because the increase in ductility which is achieved at the 2 atomic percent level is reversed and lost when the chromium is increased to the 4 atomic percent level. Further, it is clear that the 4 percent level is not effective in improving the TiAl properties even though a substantial variation is made in the atomic ratio of the titanium to the aluminum and a substantial range of annealing temperatures is employed in studying and testing the change in properties which attend the addition of the higher concentration of the additive.

## EXAMPLE 24

Samples of alloys were prepared which had a composition as follows:

Ti<sub>52</sub>Al<sub>46</sub>Cr<sub>2</sub>.

Test samples of the alloy were prepared by two different preparation modes or methods and the properties of each sample were measured by tensile testing. The

methods used and results obtained are listed in Table V immediately below.

TABLE V

| Ex. No. | Alloy No. | Composi-<br>tion<br>(at. %)                       | Process-<br>ing<br>Method | Anneal-<br>ing<br>Temper-<br>ature<br>(°C.) | Yield<br>Strength<br>(ksi) | Tensile<br>Strength<br>(ksi) | Plastic<br>Elong-<br>ation<br>(%) |
|---------|-----------|---------------------------------------------------|---------------------------|---------------------------------------------|----------------------------|------------------------------|-----------------------------------|
| 18      | 38        | Ti <sub>52</sub> Al <sub>46</sub> Cr <sub>2</sub> | Rapid Solidifi-<br>cation | 1250                                        | 93                         | 108                          | 1.5                               |
| 24      | 38        | Ti <sub>52</sub> Al <sub>46</sub> Cr <sub>2</sub> | Ingot Metall-<br>urgy     | 1225<br>1250<br>1275                        | 77<br>74<br>74             | 99<br>99<br>97               | 3.5<br>3.8<br>2.6                 |

In Table V the results are listed for alloy samples 38 which were prepared according to two Examples, 18 and 24, which employed two different and distinct alloy preparation methods in order to form the alloy of the respective examples. In addition, test methods were employed for the metal specimens prepared from the 20 alloy 38 of Example 18 and separately for alloy 38 of Example 24 which are different from the test methods used for the specimens of the previous examples.

Turning now first to Example 18 the alloy of this example was prepared by the method set forth above 25 with reference to Examples 1-3. This is a rapid solidification and consolidation method. In addition for Example 18 the testing was not done according to the 4 point bending test which is used for all of the other data reported in the tables above and particularly for Example 18 of Table IV above. Rather the testing method employed was a more conventional tensile testing according to which a metal sample is prepared as tensile bars and subjected to a pulling tensile test until the metal 30 elongates and eventually breaks. For example again with reference to Example 18 the alloy 38 was prepared into tensile bars and the tensile bars were subjected to a tensile force until there was a yield or extension of the bar at 93 ksi.

The yield strength in ksi of Example 18 of Table V compares to the yield strength in ksi of Example 18 of Table IV which was measured by the 4 point bending test. In general in metallurgical practice the yield strength determined by tensile bar elongation is a more generally accepted measure for engineering purposes.

Similarly, the tensile strength in ksi of 108 represents the strength at which the tensile bar of Example 18 broke as a result of the pulling. This measure is referenced to the fracture strength in ksi for Example 18 in Table IV. It is evident that the two different tests result in two different measures for all of the data.

With regard next to the plastic elongation here again there is a correlation between the results which are determined by 4 point bending tests as set forth in Table IV above for Example 18 and the plastic elongation in percent set forth in the last column of Table V for Example 18.

Referring again now to Table V, the Example 24 is indicated under the heading "Processing Method" to be prepared by ingot metallurgy. As used herein, the term "ingot metallurgy" refers to a melting of the ingredients of the alloy 38 in the proportions set forth in Table V and corresponding exactly to the proportions set forth for Example 18. In other words, the composition of alloy 38 for both Example 18 and for Example 24 are identically the same. The difference between the two examples is that the alloy of Example 18 was prepared by rapid solidification and the alloy of Example 24 was

prepared by ingot metallurgy. Again the ingot metallurgy involves a melting of the ingredients and solidifi-

cation of the ingredients into an ingot. The rapid solidification method involves the formation of a ribbon by the melt spinning method followed by the consolidation of the ribbon into a fully dense coherent metal sample.

In the ingot melting procedure of Example 24 the ingot is prepared to a dimension of about 2" in diameter and about  $\frac{1}{2}$ " thick in the approximate shape of a hockey puck. Following the melting and solidification of the hockey puck-shaped ingot, the ingot was enclosed within a steel annulus having a wall thickness of about  $\frac{1}{2}$ " and having a vertical thickness which matched identically that of the hockey puck-shaped ingot. Before being enclosed within the retaining ring the hockey puck ingot was homogenized by being heated to 1250° C. for two hours. The assembly of the hockey puck and containing ring were heated to a temperature of about 975° C. The heated sample and containing ring were forged to a thickness of approximately half that of the original thickness.

Following the forging and cooling of the specimen, tensile specimens were prepared corresponding to the tensile specimens prepared for Example 18. These tensile specimens were subjected to the same conventional tensile testing as was employed in Example 18 and the yield strength, tensile strength and plastic elongation measurements resulting from these tests are listed in Table V for Example 24. As is evident from the Table V results the individual test samples were subjected to different annealing temperatures prior to performing the actual tensile tests.

For Example 18 the annealing temperature employed on the tensile test specimen was 1250° C. For the three samples of the alloy 38 of Example 24, the samples were individually annealed at the three different temperatures listed in Table V and specifically 1225° C., 1250° C. and 1275° C. Following this annealing treatment for approximately two hours the samples were subjected to conventional tensile testing and the results again are listed in Table V for the three separately treated tensile test specimens.

Turning now to the test results which are listed in Table V, it is evident that the yield strengths determined for the rapidly solidified alloy are somewhat higher than those which are determined for the ingot processed metal specimens. Also, it is evident that the plastic elongation of the samples prepared through the ingot metallurgy route have generally higher ductility than those which are prepared by the rapid solidification route. The results listed for Example 24 demonstrate that although the yield strength measurements are somewhat lower than those of Example 18 they are fully adequate for many applications in aircraft engines and in other industrial uses. However, based on the

ductility measurements and the results of the measurements as listed in Table V the gain in ductility makes the alloy 38 as prepared through the ingot metallurgy route a very desirable and unique alloy for those applications which require a higher ductility. Generally speaking it is well known that processing by ingot metallurgy is far less expensive than processing through melt spinning or rapid solidification inasmuch as there is no need for the expensive melt spinning step itself nor for the consolidation step which must follow the melt spinning.

### EXAMPLE 25

Samples of an alloy containing both chromium additive and niobium additive were prepared as disclosed above with reference to Examples 1-3. Tests were conducted on the samples and the results are listed in Table VI immediately below.

TABLE VI\*

| Example Number | Alloy Number | Composition (at. %)                                               | Annealing Temperature (°C.) | Yield Strength (ksi) | Tensile Strength (ksi) | Plastic Elongation (%) | Weight Loss After 48 hrs at 98° C. (mg/cm <sup>2</sup> ) |
|----------------|--------------|-------------------------------------------------------------------|-----------------------------|----------------------|------------------------|------------------------|----------------------------------------------------------|
| 2              | 12           | Ti <sub>52</sub> Al <sub>48</sub>                                 | 1300                        | 77                   | 92                     | 2.1                    | +                                                        |
|                |              |                                                                   | 1350                        | +                    | +                      | +                      | 31                                                       |
| 15             | 78           | Ti <sub>50</sub> Al <sub>48</sub> Nb <sub>2</sub>                 | 1325                        | +                    | +                      | +                      | 7                                                        |
| 19             | 80           | Ti <sub>50</sub> Al <sub>48</sub> Cr <sub>2</sub>                 | 1275                        | +                    | +                      | +                      | 47                                                       |
|                |              |                                                                   | 1300                        | 75                   | 97                     | 2.8                    | +                                                        |
| 25             | 81           | Ti <sub>48</sub> Al <sub>48</sub> Cr <sub>2</sub> Nb <sub>2</sub> | 1275                        | 82                   | 99                     | 3.1                    | 4                                                        |
|                |              |                                                                   | 1300                        | 78                   | 95                     | 2.4                    | +                                                        |
|                |              |                                                                   | 1325                        | 73                   | 93                     | 2.6                    | +                                                        |

\*Not measured.

\*The data in this table is based on conventional tensile testing rather than on the four point bending as described above.

It is known from Example 17 in Table III above that the addition of more than one additive elements each of which is effective individually in improving and in contributing to an improvement of different properties of the TiAl compositions, that nonetheless when more than one additive is employed in concert and combination as is done in Example 17, the result is essentially negative in that the combined addition results in a decrease in desired overall properties rather than an increase. Accordingly, it is very surprising to find that by the addition of two elements and specifically chromium and niobium to bring the additive level of the TiAl to the 4 atomic percent level and employing a combination of two differently acting additives that a substantial further increase in the desirable overall property of the alloy of the TiAl composition is achieved. In fact, the highest ductility levels achieved in all of the tests on materials prepared by the Rapid Solidification Technique are those listed in the application which are achieved through use of the combined chromium and niobium additive combination.

A further set of tests were done in connection with the alloys and these tests concern the oxidation resistance of the alloys. In this test, the weight loss after 48 hours of heating at 98° C. in air were measured. The measurement was made in milligrams per square centimeter of surface of the test specimen. The results of the tests are also listed in Table VI.

From the data given in Table VI it is evident that the weight loss from the heating of alloy 12 was about 31 mg/cm<sup>2</sup>. Further, it is evident that the weight loss from the heating of alloy 80 containing chromium above was 47 mg/cm<sup>2</sup>. By contrast the weight loss resulting from the heating of the alloy 81 annealed at 1275° C. was about 4 mg/cm<sup>2</sup>. This decrease in the level of weight loss represents an increase in the oxidation resistance of the alloy. This is a very remarkable increase of about seven fold from the combination of chromium and ni-

bium additives in the alloy 81. Accordingly, what is found in relation to the chromium and niobium containing alloy is that it has a very desirable level of ductility and the highest achieved together with a very substantial improvement and level of oxidation resistance.

The oxidation test results are plotted in FIG. 4.

The strength and ductility test results of Table VI are plotted respectively in FIGS. 5 and 6.

The alloy of the present invention is suitable for use in components such as components of jet engines which display high strength at high temperatures. Such components may be for example swirlless, exhaust components, LPT blades or vanes, components vanes or ducts.

The alloy may also be employed in reinforced composite structures substantially as described in copending application Ser. No. 010,882 filed Feb. 4, 1987 and assigned to the same assignee as the subject application

the text of which application is incorporated herein by reference.

What is claimed is:

1. A chromium and niobium modified titanium aluminum alloy consisting essentially of titanium, aluminum, chromium and niobium in the following approximate atomic ratio:



2. A chromium and niobium modified titanium aluminum alloy consisting essentially of titanium, aluminum, chromium and niobium in the approximate atomic ratio of:



3. A chromium and niobium modified titanium aluminum alloy consisting essentially of titanium, aluminum, chromium and niobium in the following approximate atomic ratio:



4. A chromium and niobium modified titanium aluminum alloy consisting essentially of titanium, aluminum, chromium and niobium in the approximate atomic ratio of:



5. The alloy of claim 1, said alloy having been rapidly solidified from a melt and consolidated through heat and pressure.

6. The alloy of claim 1, said alloy having been rapidly solidified from a melt and consolidated through heat

and pressure and given a heat treatment between 1250° C. and 1350° C.

7. The alloy of claim 2, said alloy having been rapidly solidified from a melt and consolidated through heat and pressure.

8. The alloy of claim 2, said alloy having been rapidly solidified from a melt and consolidated through heat and pressure and given a heat treatment between 1250° C. and 1350° C.

9. The alloy of claim 3, said alloy having been rapidly solidified from a melt and consolidated through heat and pressure.

10. The alloy of claim 3, said alloy having been rapidly solidified from a melt and consolidated through heat and pressure and given a heat treatment between 1250° C. and 1350° C.

11. The alloy of claim 4, said alloy having been rapidly solidified from a melt and consolidated through heat and pressure.

12. The alloy of claim 4 said alloy having been rapidly solidified from a melt and consolidated through heat and pressure and given a heat treatment between 1250° C. and 1350° C.

13. A structural component for use at high strength and high temperature, said component being formed of a chromium and niobium modified titanium aluminum alloy consisting essentially of titanium, aluminum, chro-

mium and niobium in the following approximate atomic ratio:



5

14. The component of claim 13 wherein the component is a structural component of a jet engine.

15. The component of claim 13 wherein the component is reinforced by filamentary reinforcement.

16. The component of claim 15 wherein the filamentary reinforcement is silicon carbide filaments.

17. A structural component for use at high strength and high temperature, said component being formed of a chromium and niobium modified titanium alloy consisting essentially of titanium, aluminum, chromium and niobium in the following approximate atomic ratio:



18. A structural component for use at high strength and high temperature, said component being formed of a chromium and niobium modified titanium aluminum alloy consisting essentially of titanium, aluminum, chromium and niobium in the following atomic ratio:



\* \* \* \* \*

30

35

40

45

50

55

60

65